

Jan. 16, 1973

M. SCHIEKEL ET AL

3,711,383

METHOD OF MAKING CONTACT POINT COATING FOR RELAY CONTACTS

Filed Aug. 27, 1971

*FIG.1*



*FIG.2*



1

3,711,383  
**METHOD OF MAKING CONTACT POINT  
 COATING FOR RELAY CONTACTS**

Manfred Schiekel, Helmut Sussenbach, and Ingo Eichhorst, Ulm (Danube), Germany, assignors to Licentia Patent-Verwaltungs-GmbH, Frankfurt am Main, Germany

Filed Aug. 27, 1971, Ser. No. 175,626  
 Claims priority, application Germany, Aug. 28, 1970,  
 P 20 42 700.3-33  
 Int. Cl. C03b 5/50, 5/52

U.S. Cl. 204—29

4 Claims

**ABSTRACT OF THE DISCLOSURE**

A method of producing the contact point coating for a relay contact of the type wherein the contact is made of an iron-nickel alloy, e.g. as used in reed and similar type relays. A layer of gold is initially applied to the contact point of the contact and the contact is then tempered at a temperature between 700 and 1000° C. Thereafter, a layer of a two-component alloy consisting essentially of gold and either cobalt, nickel or chromium is deposited on the gold layer either galvanically or by cathode sputtering. Finally the coating may be thermally hardened by a short time further tempering at approximately 800° C. preferably in a reducing atmosphere.

**BACKGROUND OF THE INVENTION**

The present invention relates to a method for producing the coating for the contact points of relay contacts which are used for example in reed or similar relays, and the resulting relay contacts.

A relatively large number of relays with contacts enclosed in an air-tight housing operate according to the principles of reed relay developed by Bell Telephone Laboratories or very similar principles. A common characteristic feature of all of these relays is the common guiding of the magnetic and electrical flux through the contact point of the contact. The basic material for the contacting and magnetically conductive parts of such relays is generally an iron-nickel alloy of identical proportions by weight. Due to the maximum permeability  $\mu_{max}$  of this alloy being approximately  $5 \cdot 10^4$ , the magnetic conductivity thereof is suited for producing sufficiently large magnetic adhesive forces. However, the electrical properties of these alloys, i.e. the high specific resistance of  $7\Omega$  mm.<sup>2</sup>/m., the high contact resistance connected therewith and the unsatisfactory burnup properties, have made necessary the refinement of the contact giving regions or contact points and their surroundings in order to provide relays of this type which are useful for practical applications. That is, the metal at the contact points is altered or refined so that the contact points have neither high electrical nor high magnetic resistances.

The usual manner of contact refinement presently employed for this purpose is by means of the diffusion of gold. According to this process, a layer of fine gold of several micrometers thickness is deposited on the contact point of the nickel-iron basic contact material, and the gold is then diffused in a diffusion process at approximately 900° C. to a depth of 10–15  $\mu\text{m}$ . The material thus produced at the contact point is a gold-nickel-iron alloy whose concentration ratio is determined by the quantity of the gold, the temperature, and the diffusion time. These alloys are suited as contact materials but they do not represent the optimum possible for the contact material since the technical expenditures involved for producing same are very high.

2

Several sources have described contact materials on a gold base which are two-component alloys of gold and nickel, cobalt or chromium. Gold-alloy contacts for reed relays are for e.g. described in the periodical "Elektro Anzeiger," No. 15, Aug. 9, 1967, pages 9–13.

The experiments conducted by these sources have shown different travel behavior for a number of types of stresses (switching currents, switching voltage and inductance of the circuit for the various alloys). With a variation of the inductance in the circuit to be switched, a range was found in which the material moved from the anode to the cathode at the same speed as in the opposite direction; i.e. the total movement of material in this case is zero. This excellent movement of material can always be obtained for different inductances with different nickel, cobalt or chromium concentrations in the contact alloy. For gold and nickel such alloys are known to contain up to 17% by weight of nickel.

**SUMMARY OF THE INVENTION**

Based on the knowledge of these sources it is the object of the present invention to provide a method for producing contact point coatings on relay contacts of the above-mentioned type with which it is possible to apply the above-mentioned two-component alloys onto the contact points since this cannot be achieved with the conventional diffusion method.

According to the method of the present invention, a gold layer is initially applied to the contact points; the contacts are then tempered at a temperature between 700 and 1000° C.; and finally a two-component alloy of gold and cobalt, or gold and nickel, or gold and chromium, is deposited on the contact point either galvanically or by cathode sputtering.

According to a further feature of the invention, a desired thermal hardening of the contact coating material can then be accomplished by a short further tempering of the contacts at approximately 800° C. advisably in a reducing, protective gas atmosphere.

Examinations with the X-ray microprobe have shown that at these temperatures no noticeable diffusion of the gold alloy into the basic contact material takes place because of the low solubility of the contact point material or coating in the nickel-iron basic material. The rediffusion of the iron or nickel into the contact point material is so slight that no noticeable changes in the contact properties result.

**BRIEF DESCRIPTION OF THE DRAWINGS**

FIG. 1 is a sectional side view of a reed relay employing contacts with contact point coatings according to the present invention.

FIG. 2 is an enlarged partial side view of one of the contacts of FIG. 1 showing the contact point coating according to the invention.

**DESCRIPTION OF THE PREFERRED  
 EMBODIMENTS**

Referring now to FIG. 1 there is shown a reed relay including a glass vial or tube 1 having two switch or relay contacts 2 and 3 which were fused into the frontal faces 4 and 5 respectively of the glass vial 1. As is conventional in such relays, the contacts 2 and 3 are formed essentially of a ferromagnetic material. Preferably, in order to achieve proper bonding to the glass vial and to provide proper magnetic properties, the contacts 2 and 3 are formed of a nickel-iron alloy of equal proportions by weight, i.e., a mixing ratio of 50:50. Each of the contacts 2 and 3 is provided at its contact point, which is at the free end thereof, with a multilayer coating, 6 or 7 respectively according to the invention, which has neither a high electrical resistance or a high magnetic resistance.

As shown in FIG. 2 the contact paint coating 6 for the contact 2 comprises a thin layer of gold 8 which is applied directly to the surface of the nickel-iron alloy contact 2 and an overlying layer 9 of a two-component alloy of gold and nickel, cobalt or chromium. The coatings 6 and 7 may only be applied to the adjacent portions of the surfaces of the contacts 2 and 3, or may cover the entire free ends thereof if desired.

According to the method of the invention, the contact point coatings are produced by initially applying the thin layer, e.g. 0.5 to 10  $\mu\text{m}$ . thick, of gold 8 to the portion of the surface of contact 2 which is to serve as the contact point with the other contact 3. The application of this gold layer 8 may be carried out by any conventionally known process, e.g. electrolytically. The contact 2 with the gold layer 8 is then tempered by heating to a temperature between 700 and 1000° C. and then cooled. The time range for tempering may be 15 to 90 minutes. The tempering process is carried out in an atmosphere free of oxygen, e.g. in a dry nitrogen atmosphere.

After cooling, the layer 9 formed from a two-component alloy consisting of gold and a metal selected from the group consisting of cobalt, nickel and chromium is deposited on the exposed surface of gold layer 8 by conventional galvanic or cathode sputtering techniques. If galvanic deposition is utilized, the deposition occurs in a mixture bath in which the components to be deposited, i.e., gold and either cobalt, nickel or chromium, are contained. The two-component alloy layer has a preferred thickness of about 0.2 to 5  $\mu\text{m}$ .

After deposition of the two-component alloy layer 9, a desirable thermal hardening of the contact and contact point coating is then preferably carried out by a short further tempering of the contact at a temperature of approximately 800° C. This further preheating is preferably carried out in a reducing, protective gas atmosphere, e.g., a nitrogen-hydrogen gas atmosphere. At a temperature of 800° C., a tempering time of approximately two to five minutes is sufficient.

According to a preferred method of the invention the nickel-iron contact spring is covered on its contact range galvanically with a gold layer of about 4  $\mu\text{m}$ . and tem-

pered for about 40 minutes at a temperature of about 900° C. After cooling a second layer of about 2 $\mu$  thickness is galvanically deposited on this tempered gold layer. The second layer consists for example of a gold-cobalt alloy having about 5 percent cobalt. Preferably it is desired to harden this layer by means of a further tempering process of about 800° C. for about 3 minutes.

It will be understood that the above description of the present invention is susceptible to various modifications, changes and adaptions, and the same are intended to be comprehended within the meaning and range of equivalents of the appended claims.

We claim:

1. A method for producing the coating for the contact point of a relay contact such as are used in reed or similar relays wherein the relay contact is formed of an iron-nickel alloy, comprising: applying a layer of gold on the contact point; tempering the contact at a temperature between 700 and 1000° C.; and thereafter depositing a layer of a two-component alloy consisting essentially of gold and a material selected from the group consisting of cobalt, nickel and chromium, on the gold layer.
2. The method defined in claim 1 wherein said layer of a two-component alloy is deposited galvanically.
3. The method defined in claim 1 wherein said layer of a two-component alloy is deposited by cathode sputtering.
4. The method defined in claim 1 including the additional step of subsequently further thermally hardening the contact by tempering same at a temperature of approximately 800° C. preferably in a reducing atmosphere.

#### References Cited

##### UNITED STATES PATENTS

- 3,251,121 5/1966 Prival ----- 204—37 X  
3,616,281 10/1971 Head et al. ----- 204—27 X

GERALD L. KAPLAN, Primary Examiner

U.S. CL. X.R.

- 29—196; 117—71 M, 217, 234; 200—166 C; 204—27, 37, 40, 41, 192